

E. J. FOWLER AND C. KELLIE,  
REINFORCED FLANGE FOR FLANGED PRODUCTS,  
APPLICATION FILED JUNE 1, 1920.

1,407,791.

Patented Feb. 28, 1922.

2 SHEETS—SHEET 1.



FIG. 1.



FIG. 4.



FIG. 3.

INVENTORS.  
Edward J. Fowler  
Charles Kellie  
BY Book & Booth  
ATTORNEYS.

E. J. FOWLER AND C. KELLIE,  
REINFORCED FLANGE FOR FLANGED PRODUCTS.  
APPLICATION FILED JUNE 1, 1920.

1,407,791.

Patented Feb. 28, 1922.

2 SHEETS—SHEET 2.



Fig. 11.

Fig. 10.



Fig. 5.



Fig. 7.



Fig. 8.

INVENTORS:  
Edward J. Fowler  
Charles Kellie  
Booth & Booth  
ATTORNEYS.

# UNITED STATES PATENT OFFICE.

EDWARD J. FOWLER, OF REDWOOD CITY, AND CHARLES KELLIE, OF SAN FRANCISCO, CALIFORNIA, ASSIGNORS TO PACIFIC FOUNDRY COMPANY, OF SAN FRANCISCO, CALIFORNIA, A CORPORATION OF CALIFORNIA.

## REENFORCED FLANGE FOR FLANGED PRODUCTS.

1,407,791.

Specification of Letters Patent. Patented Feb. 28, 1922.

Application filed June 1, 1920. Serial No. 385,414.

To all whom it may concern:

Be it known that we, EDWARD J. FOWLER and CHARLES KELLIE, citizens of the United States, residing, the said FOWLER at Redwood City, in the county of San Mateo and State of California, and the said KELLIE at the city and county of San Francisco, State of California, have invented certain new and useful Improvements in Reenforced Flanges for Flanged Products, of which the following is a specification.

Our invention relates to flanged products, such, for example, as metal fittings comprising elbows, T's, crosses and the like; metal valves; pumps; pipes and other products having flanges.

Our invention is especially applicable to products made of relatively brittle metal or alloy, such, for example, as those alloys known as silicide irons, or high silicon acid resisting metals, used in chemical and metallurgical arts.

Due to the presence of silicon in these alloys or metals, the flanges of products made from them are not strong enough to resist the stresses of bolting, and in casting it is found that blow holes or porous spots often occur, particularly in the relatively thicker portion where the flange joins the body of the casting.

It is the object of our invention to improve said flanges in these and other respects, and to this end our invention consists in the novel reenforced flanged products which we shall hereinafter fully describe, by reference to the accompanying drawings in which—

Fig. 1 is an elevation, partly in section, showing our reenforced flanges in a T-fitting.

Fig. 2 is an elevation, partly in section, showing our reenforced flanges in an elbow fitting.

Fig. 3 is a similar elevation, showing the reenforced flange at one end of a pipe.

Fig. 4 is an end view of any of the products of Figs. 1, 2 and 3.

Fig. 5 is a face view of the front core-member.

Fig. 6 is a face view of the rear core-member.

Fig. 7 is a face view of the inner core-member.

Fig. 8 is an end view of one of the bolt-hole core-members.

55

Fig. 9 is an end view of the bore core-member.

Fig. 10 is a diametrical sectional view of the several core-members assembled, and showing the reenforcing flange-member 60 fitted therein, the dotted lines indicating the mold in which the assembled core is set in order to pour a product, such as the pipe of Fig. 3.

Fig. 11 is an elevation of the pattern from 65 which the mold is made.

In Fig. 1, the three arms of the T-fitting 1 are provided each with a flange 2 having bolt-holes 3.

At the back of each flange is the reenforcing member 4 with bolt-holes 5 registering with the bolt-holes 3 of the flange 2.

The elbow fitting 6 of Fig. 2 has similar flanges and reenforcing members, and these parts, for the sake of uniformity, are similarly identified by the numerals 2 and 4 with bolt-holes 3 and 5 respectively.

The pipe 7 of Fig. 3 is similarly flanged and its flange reenforced; and the same designating numerals are used.

A point to be noted is that the reenforcing member 4 is slightly shouldered into the fitting or pipe at the junction of flange and body, as shown at 8. This, though not essential, is advisable, in that it furnishes greater 85 stability to the union of flange and reenforcing member.

The body and flanges of the fittings of Figs. 1 and 2 of the pipe of Fig. 3 are cast from alloy or metal known in the art as silicide iron or high silicon acid resisting alloy or metal.

These silicide or silicon metals, though of varying composition, are mixtures of iron, silicon, carbon and other substances, and 95 are used for casting apparatus and parts employed in chemical and metallurgical arts on account of their acid resisting properties. But the flanges of such castings are relatively brittle and are liable to break under 100 handling in service, and especially are they weak and ill adapted to bear the stresses of bolting. They also tend to include porous spots or blow holes.

The reenforcing member 4 may be any 105 suitable metal, but that which we employ

is a plain iron casting which we shall term gray iron. It is applied to and associated with the flange in the process of casting the product, by the method which we shall presently describe.

The application of this gray iron reenforcing member to the relatively brittle silicon-iron flange of these fittings and other similar flanged products, such as pipes, valves, 10 pumps, etc., results in three marked advantages.

First, it gives additional strength to the silicon-iron flange and avoids the difficulty arising from breaking in bolting and in 15 handling in service.

Second, in the casting process the silicon iron flange is chilled when being poured against the gray-iron flange, so that there is no difficulty from porous spots or blow-holes.

Third, it closes the grain of the silicon-iron, thereby making it more acid-proof.

In order to demonstrate the practicability of manufacturing our reenforced flanged products, we offer the following as a preferred method. We first cast the gray-iron flange 4 of a thickness suitable for the purpose; then we introduce said gray-iron flange into the assembled core and bake the latter with said flange in it; then we place the core in the mold; and finally we pour the mold so that the silicon-iron flange is cast directly to the gray-iron flange.

These steps in detail, or as many of them as are required for a clear understanding, are illustrated in Figs. 5-11, and are as follows:

The gray-iron flange 4 is cast in a separate mold, by ordinary processes, and is 40 provided with correct bolt-holes.

A core is prepared to make whatever product is intended. In the present case we

have illustrated the making of a simple flanged pipe, such as shown in Fig. 3. This core comprises the following separately prepared core-members, namely, the front core-member 9 of Fig. 5, the back core-member 10 of Fig. 6, the inner core-member 11 of Fig. 7, the bolt-hole core-members 12 of Fig. 8, and the bore-core-member 13 of Fig. 9.

These several core-members are assembled into a core as shown in Fig. 10 and in the assembling the gray-iron reenforcing flange 4 previously cast is inserted and included as shown.

The assembled core of Fig. 10, with its included gray-iron flange is then baked.

A pattern 14, such as is shown in Fig. 11, is used to make the mold 15, indicated in Fig. 10, and in this mold the assembled 60 core with its included gray-iron flange is put in suitable position to make the pipe. The mold is then poured and the silicon iron flows against the gray-iron, with the results heretofore described.

We claim:—

1. Flanged products of silicon iron having a reenforcing member of iron against which the flange of said products is cast.
2. Flanged products of silicon iron having a reenforcing member of iron associated with their flanges, said member being shouldered into said product at the junction of its flange and body.
3. Flanged products having a reenforcing member against which the flange of said products is cast, said member being shouldered into said product at the junction of its flange and body.

In testimony whereof we have signed our 80 names to this specification.

EDWARD J. FOWLER.  
CHARLES KELLIE.